

Feb. 20, 1923.

1,446,213.

O. ROUCKA.

PROCESS FOR THE MANUFACTURE OF CEMENT ARTICLES AND OF REINFORCED CONCRETE MEMBERS  
AND THE LIKE.  
FILED DEC. 29, 1921.



*Fig. 1.*



*Fig. 2.*

Inventor  
*O. Roucka*  
By his Attorneys  
*Marks & Clark*

Patented Feb. 20, 1923.

1,446,213

# UNITED STATES PATENT OFFICE.

OSVALD ROUČKA, OF ROHATEC, CZECHO-SLOVAKIA.

PROCESS FOR THE MANUFACTURE OF CEMENT ARTICLES AND OF REINFORCED-CONCRETE MEMBERS AND THE LIKE.

Application filed December 29, 1921. Serial No. 525,753.

To all whom it may concern:

Be it known that I, OSVALD ROUČKA, a citizen of the Czecho-Slovakian Republic, and residing at Rohatec, Czecho-Slovakia, have invented certain new and useful Improvements in and Relating to a Process for the Manufacture of Cement Articles and of Reinforced-Concrete Members and the like (for which I have filed applications in Great Britain, No. 31,636, dated November 25th, 1921; Czecho-Slovakia, application filed July 19th, 1921; in Italy, August 12th, 1921; in France, August 12th, 1921; in Austria, September 9th, 1921; and in Germany, September 10th, 1921), of which the following is a specification.

While it has already been proposed to use steam and hot air for hardening articles made of cement, the processes made known hitherto have not given satisfactory results, as, when using hot air, a satisfactory degree of hardness was not obtained, when hardening by means of steam not under pressure, the hardening took too long and, when hardening by means of steam under pressure, cracks and deformations in the surface of the articles appear, the surface scales off and the appearance of the articles suffers through the condensed water vapour.

These disadvantages are obviated by the process according to the present invention, according to which the articles are first pre-heated to about 60-80° C., whereupon the temperature and pressure are increased by admitting steam under pressure. The process according to the invention is as follows:—

In the drawings there is shown an apparatus by which the process may be carried out and in which:—

Fig. 1 is a side elevational view of the apparatus, and

Fig. 2 is an end elevational view thereof. Similar characters of reference are employed to indicate corresponding parts throughout the views.

The cement or concrete articles are placed in a vessel 1, which has been tested to about 8 atmospheres. The vessel is preferably of an elongated cylindrical shape being removably closed by the flange cover 2. When the vessel is closed, the heating system generally designated by the numeral 3 and having its main portion arranged at the bottom of the vessel is put in operation, so

that the temperature rises by 1° to 5° per minute. At each rise of temperature by about 10° C. a certain amount of steam can be admitted into the vessel 1 for raising the degree of humidity. After a temperature of from 60° to 80° C. has been reached, according to the water content and the composition of the cement used, the further increase in temperature is continued at a considerably slower rate than that given above, namely, by about 0.1° to 1° in each minute by the combined action of the heating system 3 and the admitted steam or only by the action of steam, until the pressure in the vessel reaches about 7 to 13 atmospheres. When hardening articles having a considerable water content, superheated steam is preferably used. When a pressure of about from 7 to 13 atmospheres has been reached in the vessel 1, the manufactured articles are left in this pressure from 8 to 10 hours, according to the kind of article treated, after which the hardening will be complete.

The heating system 3 which is associated with the vessel has its main portion, including a perforated pipe 4 preferably mounted at the bottom of the vessel. Steam is admitted over the entire length of the vessel. The vessel is fitted at its lowest point with a valved outlet pipe 5 for draining off the water of condensation and at the top with a steam outlet valve 6. The other fittings of the vessel comprise a pressure gauge 7, a thermometer 8 on the cover for indicating the internal temperature of the vessel and the usual safety valves 9.

The process according to the invention has the following advantages:—

(1) The articles treated are given a high compressive strength within a few hours, which, for instance in the case of concrete articles exceeds 600 kg. to 1 sq. cm.

(2) The adhesion of the iron reinforcement of reinforced concrete members considerably exceeds the normal adhesion.

(3) The manufacture of articles does not depend on the atmospheric conditions.

(4) A considerable amount of space is saved.

(5) There is also a saving in work and material, as the articles show great strength with a relatively low percentage of cement and for instance in the case of roof tiles the supports and the repeated smoothing

over are not required, so that the roof tiles can be made thinner and consequently lighter.

(6) Mass production is made possible and building material becomes considerably cheaper.

(7) It becomes possible to ascertain the state of the cement within a few hours.

What I claim is:—

- 10 1. A process for the manufacture of cement articles and of reinforced concrete members and the like, consisting in this that the raw material is hardened in an enclosed vessel, the temperature in the interior of the vessel being first brought to a temperature of about 60-80° C. at a rate of about 1 to 5° C. per minute, whereupon the further increase in temperature is continued more slowly at a rate of 0.1 to 1° C. per minute,
- 15 20 ute, the pressure being at the same time increased until the pressure rises to about 7 to 13 atmospheres, whereupon the articles are left for about 8 to 10 hours under this pressure, as set forth.

2. A process for the manufacture of cement articles and of reinforced concrete members and the like, consisting in this that the raw material is hardened in an enclosed vessel by means of steam and that by means of a heating system the temperature in the interior of the vessel is first brought to a temperature of about 60-80° C. at a rate of about 1 to 5° C. per minute, whereupon the further increase in temperature is continued more slowly at a rate of 0.1 to 1° C. per minute, the pressure being at the same time increased by the regulated admission of steam until the pressure rises to about 7 to 13 atmospheres, whereupon the articles are left for about 8 to 10 hours under this pressure, as set forth.

In testimony whereof I have signed my name to this specification.

OSVALD ROUČKA.

Witnesses:

LANDISK KNOT,  
FREY HOVOMIL MATHAUSER.